

## UNITED STATES PATENT OFFICE

2,467,675

## ALLOY OF HIGH DENSITY

Jacob Kurtz, Teaneck, and Harold G. Williams,  
Ramsey, N. J., assignors to Callite Tungsten  
Corporation, Union City, N. J., a corporation of  
Delaware

No Drawing. Original application September 30,  
1942, Serial No. 460,226. Divided and this ap-  
plication March 10, 1943, Serial No. 478,610

8 Claims. (Cl. 75—22)

1

The present invention relates to alloys of refractory metals, such as tungsten, molybdenum, rhenium, and tantalum. More particularly, it relates to alloys of such metals that are of high density and free from the usual porosity and intergranular voids that are characteristic of alloys made by the methods of powder metallurgy heretofore practised.

In our copending application Serial No. 460,226, of which this application is a division, a method of making an alloy of refractory metals such as tungsten, molybdenum, rhenium and tantalum is disclosed. This alloy has a density approximating the theoretical density of the refractory metals referred to when they have been hot swaged, and contains grain refining additions which control the grain size and structure of the alloy and give certain other characteristics thereto. The alloy of the present invention contains no grain refining additions but nevertheless it has a density approximating the theoretical density of the swaged refractory metals contained therein.

According to methods commonly in use, tungsten or molybdenum and similar refractory metals having high melting points are usually worked from their powders. For instance, tungsten or molybdenum metal powder is placed in a die and compressed under high pressure until it is formed into the shape desired, such as a rod or ingot. It is then presintered, that is, sintered at a temperature and for such a period of time that the article is strong enough to be handled for further treatment. Further treating and sintering at temperatures equal to approximately 90% of the fusing current for the particular rod or ingot, further shrinks and strengthens the rod or ingot. The treated ingot, however, is still quite porous and has many intergranular voids, the density at this stage being approximately 17-18 grams per cubic centimeter in the case of tungsten.

The rod or ingot must then be hot swaged until it is further compacted whereby the density increases rapidly from the values of 17-18 to a value approximately 19.3 for fully swaged rods, having a reduction in area of 80-90%. This density is generally referred to as the theoretical density.

According to the method of the present invention, purified refractory metal powder, such as tungsten or molybdenum, having a particle size of approximately from 1 to 25 microns, is combined with a small but effective amount of powdered metals that result in the alloying, bonding and densifying of the rod or ingot without the necessity of swaging. These alloying metals are formed from an appropriate selection

that are more properly described as alloying metals, and a second group consisting of the noble metals. In the first group are manganese, iron, cobalt and nickel, and in the second group, platinum, palladium, gold, osmium, iridium, ruthenium and rhodium.

This alloying, bonding and densifying metal consists of a mixture of finely divided metal powders approximately one-half by weight of base metal and the balance noble metal. After these two constituents are thoroughly mixed they are added to the refractory metal powder in the proportion of approximately .25%—4% by weight, thoroughly ball-milled and mixed to assure uniform distribution of the densifying metal throughout the refractory metal. The mixture is then ready for pressing into formed pieces, discs, and the like, and subsequent heat treatment at a temperature of 1500-2000° C. in a hydrogen or neutral atmosphere or even in a high frequency vacuum furnace, using a molybdenum or tungsten tube or elongated crucible.

The following example illustrates the method of forming this alloy:

## Example

First, the alloying, bonding and densifying metal mixture is prepared. Approximately equal proportions by weight of pure finely divided 30 nickel powder, and pure finely divided platinum powder are thoroughly mixed and ball-milled. Platinized nickel powder (containing approximately 50% by weight of platinum) made by shaking nickel powder in a solution of chlor-platinic acid may be used. Then, approximately 1/2% by weight of this prepared mixture is added to finely divided tungsten powder of a particle size of 1-25 microns and is thoroughly mixed. It may be ball-milled for a period of several hours, 40 or at least long enough to assure the uniform distribution of the small amount of alloying powders throughout the mass of tungsten powder.

This mixture is then ready for pressing in a 45 suitable mold either in a tablet machine, or in a conventional hydraulic press, depending on the size and shape of the desired finished piece. After pressing, the formed pieces are then heat treated in an electric furnace at a temperature of 1500-1850° C. in a dry hydrogen atmosphere for about one hour, the time depending, of course, on the size, shape and number of pieces inserted into the hot zone, and the characteristics of the furnace.

55 After this heat treatment, the pieces have been fully sintered and shrunk in volume in a uniform manner maintaining in a characteristic way all the sharp contours of the pieces. The volume

shrinkage will vary from about 15-25% of the original volume depending on pressures and sintering temperatures used. With  $\frac{1}{4}\%$  Ni and  $\frac{1}{4}\%$  Pt, 99.5% tungsten, densities are obtained without swaging as high as 19.35 grams per cubic centimeter, comparable to the density of a piece of hot swaged tungsten rod of 19.3.

This high density is an indication of a fully sintered body exceptionally free from porosity and intergranular voids. The micro-structure confirms this, and shows a well ordered, well developed, fairly large grained crystal structure.

An alternate method of adding the nickel and platinum in the above example may be employed with equally satisfactory results. Standard stock solutions of the soluble salts or compounds, or the metals to be added, are made up. The salts chosen belong to the class which when completely dehydrated are easily decomposable to their metallic states when heated in a reducing atmosphere. Examples of such are the acetates, chlorides, and nitrates of iron, cobalt, nickel and manganese; chloroplatinic acid, ammonium chloroplatinate, gold chloride, and similar compounds of the other metals used. A measured amount of the solution of the base metal and the noble metal is added to the oxide of the refractory metal, thoroughly dried in a manner to assure uniform distribution of the salts, and subsequently this mixture is reduced in the usual manner to metal powder. Or the solutions may be added to the refractory metal powder forming a slurry, care being taken to mix and stir the powder thoroughly to get uniform distribution of the metallic salts added. The slurry is carefully dried with constant stirring, and, when dry, it is sieved to break up any lumpy formation, put into a nickel boat and run through a reduction furnace to insure complete reduction to their metallic states. The powders are then sieved through 200 mesh and are now ready for pressing into any desired form or shape.

While the example given above illustrates the method of making the dense alloy of the invention with tungsten as the refractory metal, it will be understood that a similar method of alloying molybdenum, rhenium and tantalum also comes within the scope of the invention. In the case of molybdenum, however, about 1% of the alloying, bonding and densifying metals should be added.

The alloys of the invention are extraordinarily suitable for making the face plates of contact points and may be used for making large shaped objects such as crucibles and cylinders, both solid and hollow. They may, in fact, be used wherever hard, strong, dense metal capable of withstanding high temperatures is desired.

Subsequent heating at approximately 600°-1000° C. for periods of about 1-10 hours will cause precipitation hardening whenever desired.

Having thus described our invention, what we claim is:

1. A pressed and sintered alloy of high density consisting of a refractory metal of the group consisting of tungsten, molybdenum, rhenium and tantalum having a particle size of from 1 to 25 microns and from 0.25% to 4% by weight of a mixture of finely divided alloying, bonding and densifying metal consisting of 50% by weight of a metal of the group consisting of manganese, iron, cobalt and nickel, and 50% by weight of a metal of the group consisting of platinum, palladium, gold, osmium, iridium, ruthenium and rhodium, said alloy having a density approximating the theoretical density of said included refractory metal when swaged hot.

2. A pressed and sintered alloy of high density consisting of 99.50% tungsten having a particle size of from 1 to 25 microns, 0.25% of nickel and 0.25% of platinum, said alloy having a density approximating the theoretical density of hot swaged tungsten.

3. A pressed and sintered alloy of high density consisting of 99% of tungsten having a particle size of from 1 to 25 microns, 0.50% of nickel and 0.50% of platinum, said alloy having a density approximating the theoretical density of hot swaged tungsten.

4. A pressed and sintered alloy of high density consisting of 99% of molybdenum having a particle size of from 1 to 25 microns, 0.50% of nickel and 0.50% of platinum, said alloy having a density approximating the theoretical density of hot swaged molybdenum.

5. A pressed and sintered alloy of high density consisting of 99% of a refractory metal of the group consisting of tungsten, molybdenum, rhenium and tantalum having a particle size of from 1 to 25 microns, 0.50% of nickel and 0.50% of a metal of the group consisting of platinum, palladium, gold, osmium, iridium, ruthenium and rhodium, said alloy having a density approximating the theoretical density of the included refractory metal when hot swaged.

6. A pressed and sintered alloy consisting of a powdered refractory metal of the group consisting of tungsten and molybdenum, and a mixture of nickel and platinum; said mixture consisting of 50% by weight of nickel and 50% by weight of platinum, said refractory metal being present in an amount of at least 96% by weight of the alloy, and said mixture being present in an amount sufficient to produce a dense product and up to 4% by weight of the alloy.

7. A pressed and sintered alloy consisting of a powdered refractory metal of the group consisting of tungsten and molybdenum, and a mixture of two metals, one metal selected from the group consisting of iron, cobalt and nickel and the other metal selected from the group consisting of platinum and palladium, said refractory metal being present in an amount of at least 96% by weight of the alloy, said mixture containing substantially equal parts of each of the metals of the mixture, being present in an amount sufficient to produce a dense product and constituting the balance of the alloy.

8. A pressed and sintered alloy consisting of a powdered refractory metal of the group consisting of tungsten and molybdenum, and a mixture of nickel and palladium, said refractory metal being present in an amount of at least 96% by weight of the alloy, said mixture containing substantially equal parts of nickel and palladium, being present in an amount sufficient to produce a dense product and constituting the balance of the alloy.

JACOB KURTZ.  
HAROLD G. WILLIAMS.

#### REFERENCES CITED

The following references are of record in the file of this patent:

#### UNITED STATES PATENTS

| 70 | Number    | Name      | Date          |
|----|-----------|-----------|---------------|
|    | 2,157,935 | Hensel    | May 9, 1939   |
|    | 2,157,936 | Hensel    | May 9, 1939   |
|    | 2,183,359 | Smithells | Dec. 12, 1939 |
|    | 2,188,405 | Hensel    | Jan. 30, 1940 |